



US007829138B2

(12) **United States Patent**  
**Masuda et al.**

(10) **Patent No.:** **US 7,829,138 B2**  
(45) **Date of Patent:** **Nov. 9, 2010**

(54) **METAL MATERIAL FOR PARTS OF  
CASTING MACHINE, MOLTEN ALUMINUM  
ALLOY-CONTACT MEMBER AND METHOD  
FOR PRODUCING THEM**

(75) Inventors: **Jun Masuda**, Mishima (JP); **Shuhei Homma**, Numazu (JP); **Ryousuke Fujimoto**, Numazu (JP)

(73) Assignee: **Toshiba Kikai Kabushiki Kaisha**, Tokyo-To (JP)

(\*) Notice: Subject to any disclaimer, the term of this patent is extended or adjusted under 35 U.S.C. 154(b) by 0 days.

(21) Appl. No.: **10/599,118**

(22) PCT Filed: **Mar. 22, 2005**

(86) PCT No.: **PCT/JP2005/005100**

§ 371 (c)(1),  
(2), (4) Date: **Sep. 20, 2006**

(87) PCT Pub. No.: **WO2005/090637**

PCT Pub. Date: **Sep. 29, 2005**

(65) **Prior Publication Data**

US 2007/0196684 A1 Aug. 23, 2007

(30) **Foreign Application Priority Data**

Mar. 22, 2004 (JP) 2004-082990

(51) **Int. Cl.**  
**B05D 5/08** (2006.01)  
**B05D 5/00** (2006.01)

(52) **U.S. Cl.** 427/180; 427/202; 427/205;  
427/374.6; 427/376.6

(58) **Field of Classification Search** ..... None  
See application file for complete search history.

(56) **References Cited**

**U.S. PATENT DOCUMENTS**

|                   |        |                             |
|-------------------|--------|-----------------------------|
| 3,495,630 A       | 2/1970 | Hansen et al.               |
| 4,868,069 A *     | 9/1989 | Darrow ..... 428/610        |
| 4,995,427 A       | 2/1991 | Berchem                     |
| 4,996,114 A *     | 2/1991 | Darrow ..... 428/610        |
| 2005/0116192 A1   | 6/2005 | Vincent                     |
| 2007/0144627 A1 * | 6/2007 | Masuda et al. ..... 148/519 |
| 2007/0196684 A1   | 8/2007 | Masuda et al.               |

**FOREIGN PATENT DOCUMENTS**

EP 06 65 598 2/1996

(Continued)

**OTHER PUBLICATIONS**

JP 2001-342530 English Machine Translation, Honma et al., Dec. 2001.\*

(Continued)

*Primary Examiner*—Jennifer C McNeil

*Assistant Examiner*—Jason L Savage

(74) *Attorney, Agent, or Firm*—DLA Piper LLP US

(57) **ABSTRACT**

A Ni alloy layer is formed on a surface of a steel base on the side to be in direct contact with a molten aluminum alloy, and titanium carbide (TiC) is bonded in a particulate state to the surface of the Ni alloy layer. This makes it possible to provide a metal material having materially enhanced melting loss resistance without resorting to conventional techniques, such as the provision of a ceramic coating by PVD or CVD.

**4 Claims, 3 Drawing Sheets**



## FOREIGN PATENT DOCUMENTS

|    |               |         |
|----|---------------|---------|
| EP | 06-95-998     | 2/1996  |
| JP | 51-20303      | 6/1976  |
| JP | 03-126681     | 5/1991  |
| JP | 07-001077     | 1/1995  |
| JP | 08-025063     | 1/1996  |
| JP | 08-132215     | 5/1996  |
| JP | 08-229657     | 9/1996  |
| JP | 2000-351054   | 12/2000 |
| JP | 2001-287004   | 10/2001 |
| JP | 2001-300711   | 10/2001 |
| JP | 2001-342530   | 12/2001 |
| JP | 2002-066708   | 3/2002  |
| JP | 2003-170262   | 6/2003  |
| JP | 2005-264306   | 9/2005  |
| KR | 10-1987-11269 | 12/1987 |

## OTHER PUBLICATIONS

JP 2001-300711 English Machine Translation, Negishi, Oct. 2001.\*  
 JP 08-229657 English Machine Translation, Nakayama et al., Sep. 1996.\*  
 JP 76020303, Nippon Tungsten KK, Jun. 1976, Titanium Carbide Cement Scraping Tool Formed as a Nitrided Layer on Steel Substrate, English Abstract from DWPI Database.\*  
 English International Preliminary Exam Report for PCT/JP2005/00510, Jan. 2007.\*  
 Office Action issued in U.S. Appl. No. 11/565,771, mailed Oct. 28, 2008.  
 Notice of Allowance issued in related Korean Patent Application No. 2006-0118288 mailed Apr. 4, 2008.  
 English language abstract of JP 03-126681, published May 29, 1996.  
 Machine English language translation of 08-025063, published Jan. 30, 1996.  
 Machine English translation of JP 2001-287004, published Oct. 16, 2001.

English language abstract of KR 10-1987-0011269, published Dec. 22, 1987.  
 International Preliminary Examination Report issued in International Application No. PCT/JP2005/005100, mailed Mar. 22, 2005.  
 International Search Report of PCT/JP2007/056048.  
 English Language Abstract for JP 2005 264306.  
 English Language translation of JP-2005-264306.  
 English Language Abstract for JP 2000 351054.  
 English Language translation of JP-2000-351054.  
 English Language Abstract for JP 2002 066708.  
 English Language translation of JP-2002-066708.  
 English Abstract of JP 08-025063.  
 English Abstract of JP 2001-287004.  
 English language translation of International Preliminary Report on Patentability issued in Application No. PCT/JP07/056048 mailed Nov. 13, 2008.  
 International Search Report issued in PCT/JP05/05100 on Jul. 5, 2005.  
 Japanese Office Action issued in Application No. 2004-82990 mailed Apr. 7, 2009.  
 English Translation of Japanese Office Action issued in Application No. 2004-82990 mailed Apr. 7, 2009.  
 Machine English language translation of JP 07-001077, published Jan. 6, 1995.  
 English Abstract of JP 07-001077.  
 Machine English language translation of JP 2003-170262, published Jun. 17, 2003.  
 English Abstract of JP 2003-170262.  
 Machine English language translation of JP 08-132215, published May 28, 1996.  
 English Abstract of JP 08-132215.  
 US Office Action issued in related U.S. Appl. No. 11/565,771 dated Jun. 24, 2009.  
 Office Actions issued in U.S. Appl. No. 11/565,771 on Dec. 7, 2009.  
 Office Action issued in U.S. Appl. No. 11/565,771 on Jun. 30, 2010.

\* cited by examiner



FIG. 1



FIG. 2



FIG. 3

EXAMPLE 1  
TiN (CVD)EXAMPLE 2  
TiC PERTICLEEXAMPLE 3  
TiC PERTICLE + BN

FIG. 4



F I G. 5

## 1

**METAL MATERIAL FOR PARTS OF  
CASTING MACHINE, MOLTEN ALUMINUM  
ALLOY-CONTACT MEMBER AND METHOD  
FOR PRODUCING THEM**

TECHNICAL FIELD

The present invention relates to a metal material for parts of a casting machine, a molten aluminum alloy-contact member and a method for producing them, and more particularly to a metal material for parts of a casting machine and a molten aluminum alloy-contact member, which have excellent melting loss resistance to a molten aluminum alloy, and a method for producing them.

BACKGROUND ART

A molten aluminum alloy has a property of reacting with a metal, such as iron, to produce an intermetallic compound. Those steel parts of a casting machine which are in direct contact with a molten aluminum alloy can be damaged due to their reaction with aluminum. This phenomenon is called melting loss. In casting of an aluminum alloy, it is essential to take measures against melting loss for chief parts, such as a conduit, a mold, a sleeve and an insert, which are to contact a molten aluminum alloy.

A steel material, such as a tool steel which has undergone a nitriding treatment, is generally used for a mold, etc. for use in aluminum casting. The nitriding treatment, which comprises diffusing nitrogen from a steel surface to form a hard nitride layer, is excellent in enhancing the wear resistance of the material. It has been pointed out, however, that such treatment is not always sufficient for preventing a melting loss.

With respect to members for which high melting loss resistance is required, it is a common practice to form a ceramic coating on the surface of a member by a vapor deposition method, such as PVD (physical vapor deposition) or CVD (chemical vapor deposition). Such a ceramic coating is known to be chemically stable to a molten aluminum alloy and exhibit very high melting loss resistance (see New Mechanical Engineering Handbook, B2, Processing/Processing Devices, p. 157).

The biggest problem with a ceramic coating, as formed by PVD or CVD, is peeling due to a thermal stress. In particular, because of a large difference in thermal expansion coefficient between a steel base and a ceramic coating, a large thermal stress will be produced at the boundary between the ceramic coating and the steel base by the repetition of heating and cooling during successive casting cycles. The large thermal stress often causes peeling of the ceramic coating from the base, whereby the base comes into direct contact with a molten aluminum alloy. Melting of the steel base thus begins suddenly, resulting in a melting loss of the base.

For the purpose of preventing such peeling of ceramic coating, various improvements have been made in methods for forming ceramic coatings in order to reduce the thickness of a coating, thereby minimizing a thermal stress generated at the boundary between the coating and a base, or to enhance the bonding strength between a coating and a base.

Despite the various improvements, however, the fundamental difference in thermal expansion between a ceramic coating and a steel base has been an insurmountable bar, and complete prevention of peeling of a ceramic coating has not been achieved as yet.

It is therefore an object of the present invention to solve the above problems in the prior art and provide a metal material

## 2

for parts of a casting machine and a molten aluminum alloy-contact member, which have materially enhanced melting loss resistance, without resorting to conventional techniques, such as the provision of a ceramic coating by PVD or CVD.

It is another object of the present invention to provide a method for producing a molten aluminum alloy-contact member, which makes it possible to strongly bond TiC particles to a Ni alloy layer of the member so that the member has materially enhanced melting loss resistance.

DISCLOSURE OF THE INVENTION

In order to achieve the above objects, the present invention provides a metal material for machine parts for use in a casting machine for casting an article from a molten aluminum alloy, comprising a steel base, a Ni alloy layer formed on a surface of the base, and titanium carbide (TiC) bonded in a particulate state to the surface of the N alloy layer.

The present invention also provides a machine part for use in a casting machine for casting an article from a molten aluminum alloy, comprising a body, composed of a steel base and a nickel alloy layer formed on a surface of the base on the side to be in direct contact with a molten aluminum alloy, and titanium carbide (TiC) bonded in a particulate state to the surface of the Ni alloy layer.

The present invention also provides a method for producing a molten aluminum alloy-contact member for use in a casting machine for casting an article from a molten aluminum alloy, comprising the steps of: forming a Ni alloy layer on a surface of a steel base, thereby forming a body; burying the body in TiC powder; and placing the body, together with the TiC powder, in a vacuum heating oven and heating them under vacuum to a temperature at which a liquid phase generates from the Ni alloy, thereby bonding the TiC particles to the surface of the Ni alloy layer.

According to the present invention, a molten aluminum alloy-contact member, having materially enhanced melting loss resistance, can be provided without resorting to conventional techniques, such as the provision of a ceramic coating by PVD or CVD. Thus, by applying the present invention to those parts of a casting machine which are to be in direct contact with a molten aluminum alloy, the lives of the parts can be considerably extended.

BRIEF DESCRIPTION OF THE DRAWINGS

FIG. 1 is a schematic diagram showing the structure of a metal material for parts of a casting machine, according to an embodiment of the present invention;

FIG. 2 is a schematic diagram showing the structure of a metal material for parts of a casting machine, according to another embodiment of the present invention;

FIG. 3 is a diagram illustrating a method for producing a molten aluminum alloy-contact member according to the present invention;

FIG. 4 is a graphical diagram showing the results of a melting loss test carried out for molten aluminum alloy-contact member specimens prepared in Examples; and

FIG. 5 is a photograph showing the structure of a molten aluminum alloy-contact member produced in Examples.

BEST MODE FOR CARRYING OUT THE  
INVENTION

Preferred embodiments of the present invention will now be described with reference to the drawings.

FIG. 1 is a diagram schematically showing the structure of a metal material for parts of a casting machine, according to an embodiment of the present invention. The metal material of this embodiment comprises a steel base, a Ni alloy layer formed on the base, and titanium carbide (TiC) bonded in a particulate state to the surface of the Ni alloy layer.

TiC particles have a property of repelling a molten aluminum alloy. By utilizing this property, direct contact of a molten aluminum alloy with the steel base can be prevented and high melting loss resistance can be achieved.

Unlike the mechanism of enhancing the melting loss resistance of a metal material by covering the entire surface with a coating to shut off contact of a molten aluminum alloy with the base metal surface, as in the conventional ceramic coating by PVD or CVD, the present metal material can be provided with materially enhanced melting loss resistance simply by densely scattering TiC particles over the base metal surface.

In the structure that the TiC is bonded in a particular state to the Ni alloy layer, a large thermal stress will not act on the TiC particles even when the base thermally expands or contracts. Thus, the TiC particles hardly peel off and, therefore, the melting loss resistance can be maintained for a long period.

The TiC particles may be partly exposed on the surface of the Ni alloy layer. This can increase the contact angle with a molten aluminum alloy, thereby enhancing the property of repelling the molten aluminum alloy.

Preferably, the gaps in the TiC particles are filled in with fine ceramic particles comprising at least one of boron nitride (BN), alumina ( $Al_2O_3$ ) and zirconia ( $ZrO_2$ ), as shown in FIG. 2. The fine ceramic particles improve the melting loss resistance of the underlying Ni alloy layer to which the TiC particles are bonded.

The Ni alloy preferably has the composition of 2.6 to 3.2% of B, 18 to 28% of Mo, 3.6 to 5.2% of Si and 0.05 to 0.22% of C, with the remainder being Ni and unavoidable impurities.

The TiC particles can be bonded to the Ni alloy, having the above composition, with high strength through generation of a liquid phase from the Ni alloy. Further, because of good wetting between the liquid phase and TiC particles, a large number of TiC particles can be densely bonded to the Ni alloy layer.

A conduit, a mold, a molten metal sleeve, an insert, etc. for use in a casting machine, can be typically exemplified for molten aluminum alloy-contact members or machine parts of a casting machine to which the above-described metal material is applicable.

FIG. 3 illustrates a method for producing a molten aluminum alloy-contact member according to an embodiment of the present invention.

The member to be produced comprises a steel base. First, a Ni alloy layer is formed on the base by thermal spraying.

Next, as shown in FIG. 3(a), a vessel containing TiC powder is prepared, and the member composed of the base and the Ni alloy layer is entirely varied in the TiC powder.

The vessel, containing the TiC powder and the member buried in it, is placed in a vacuum heating oven, and heated under vacuum to a temperature at which a liquid phase is generated from the Ni alloy, thereby bonding the TiC particles to the surface of the Ni alloy layer.

By the heating, the TiC particles are bonded to the Ni alloy layer in such a state that they protrude from the surface of the Ni alloy layer, as shown in FIG. 3(b). In this connection, it is undesirable if the TiC particles become entirely covered with the melting Ni alloy in the heating process. In order not to entirely cover the TiC particles with the Ni alloy but to strongly bond the TiC particles to the Ni alloy layer with the

particles partly exposed on the surface of the Ni alloy layer, the average particle diameter of the TiC particles is preferably made 10 to 500  $\mu m$ .

When the particle diameter of the TiC particles is smaller than 10  $\mu m$ , it is difficult to control the temperature during the vacuum-heating so that the TiC particles may not be entirely covered with the liquid phase of the Ni alloy. The intended melting loss resistance will not be obtained if the TiC particles are entirely covered with the liquid phase of the Ni alloy.

When the particle diameter of the TiC particles is larger than 500  $\mu m$ , on the other hand, the liquid phase of the Ni alloy will cover only lower portions of the particles with small contact area and weak bonding strength. Accordingly, the particles will easily fall off.

After the bonding of TiC particles to the member, the member may optionally be subjected to a process comprising applying a slurry of a mixture of a binder and a fine ceramic powder comprising at least one of boron nitride (BN), alumina ( $Al_2O_3$ ) and zirconia ( $ZrO_2$ ) to the TiC particles, and burning the ceramic powder into the surface of the member. The melting loss resistance of the member increases after this process.

The Ni alloy layer, to which the TiC particles are bonded, itself has a poor melting loss resistance to a molten Al alloy. The melting loss resistance can be improved by attaching the fine ceramic powder to the Ni alloy layer. Furthermore, the attached fine powder is present such that it fills in the gaps in the TiC particles. Accordingly, the fine ceramic powder hardly falls off upon contact with a molten aluminum alloy.

## EXPERIMENTAL EXAMPLES

The present invention will now be further described with reference to experimental examples.

In the examples, test specimens for melting loss test were prepared using a steel material (JIS S45C) as a base. A Ni alloy having the above-described composition was thermally sprayed onto the steel base to line the base with the Ni alloy. The Ni alloy-lined base was then buried in TiC powder in a vacuum heating oven, and heated under vacuum until the TiC particles came to be bonded to a liquid phase generated from the Ni alloy.

Two types of test specimens were prepared for Example 1 and Example 2. The specimen of Example 1 is the above specimen with the TiC particles bonded thereto but no ceramic powder attached, while the specimen of Example 2 was prepared by burning fine powder of boron nitride (BN) into the surface of the above specimen with the TiC particles bonded thereto.

For comparison with the melting loss resistances of the specimens of Examples 1 and 2, a comparative specimen was prepared by coating the same steel base as in Examples 1 and 2 with titanium nitride (TiN) by CVD.

A melting loss test was carried out in the following manner: Each test specimen was immersed in a molten aluminum alloy (JIS AC4C) which was kept at 720° C., and was rotated at a peripheral speed of 0.8 m/s while keeping it immersed in the molten metal for 24 hours. Thereafter, the test specimen was taken out of the molten metal, and a change in the weight of the specimen was measured. FIG. 4 is a graph showing the results of the melting loss test. In the graph of FIG. 4, the abscissa shows the amount of melting loss per unit area ( $mg/cm^2$ ) for each of the specimens of Examples 1 and 2 and for the comparative specimen.

As is apparent from comparison of the data for the specimen of Example 1 with the data for the comparative specimen, the amount of melting loss for the specimen of Example

1, having the TiC particles bonded to the Ni alloy layer, can be reduced to approximately half of the amount of melting loss for the comparative specimen having the TiN coating formed by CVD. The data in FIG. 4 also shows no melting loss for the specimen of Example 2, having the fine BN powder filled in the gaps in the TiC particles, thus indicating superiority of the specimen of Example 2 to the specimen of Example 1.

A description will now be given of Example 3 in which a conduit, a flow passage for a molten aluminum alloy, was produced as a molten aluminum alloy-contact member.

In Example 3 was used the same material as in Example 2 except for using fine alumina powder having an average particle diameter of about 1  $\mu\text{m}$  instead of the fine boron nitride (BN) powder. FIG. 5 shows a photograph of a cross-section of the material of Example 3. As can be seen in the photograph, a large number of TiC particles having a size of about 100  $\mu\text{m}$  are bonded to the surface of the Ni alloy layer.

For comparison with the melting loss resistance of the conduit of Example 3, a comparative conduit was produced using a material composed of the same steel base and a coating of TiN formed by CVD. A molten aluminum alloy at about 700° C. was allowed to flow in the conduit of Example 3 and in the comparative conduit, and the time elapsed before detection of a melting loss was measured.

A melting loss was detected after about 19 hours in the comparative conduit, whereas no melting loss was detected in the conduit of Example 3 even after an elapse of 100 hours.

The invention claimed is:

1. A method for producing a molten aluminum alloy-contact member for a casting machine for casting an article from a molten aluminum alloy, comprising the steps of:

forming a Ni alloy layer on a surface of a steel base, thereby forming a body;  
burying the body in TiC powder; and  
placing the body, together with the TiC powder, in a vacuum heating oven and heating them under vacuum to a temperature at which a liquid phase generates from the Ni alloy, thereby densely bonding the TiC particles to the surface of the Ni alloy layer, the TiC particles repelling molten aluminum alloy.

2. The method for producing a molten aluminum alloy-contact member according to claim 1, wherein after the bonding of the TiC particles to the Ni alloy layer, the member is subjected to a process comprising applying a slurry of a mixture of a binder and a fine ceramic powder comprising at least one of boron nitride (BN), alumina ( $\text{Al}_2\text{O}_3$ ) and zirconia ( $\text{ZrO}_2$ ) to the TiC particles, and burning the ceramic powder into the surface of the member.

3. The method for producing a molten aluminum alloy-contact member according to claim 1, wherein the average particle diameter of the TiC powder is in the range of 10-500 nm.

4. The method for producing a molten aluminum alloy-contact member according to claim 1, wherein the Ni alloy layer is formed by thermal spraying of a Ni alloy having the composition of 2.6 to 3.2% of B, 18 to 28% of Mo, 3.6 to 5.2% of Si and 0.05 to 0.22% of C, with the remainder being Ni and unavoidable impurities.

\* \* \* \* \*